

Oct. 21, 1969

R. V. SARA

3,473,900

ALUMINUM-CARBON FIBER COMPOSITES

Filed Feb. 21, 1967



INVENTOR  
RAYMOND V. SARA  
BY *Richard J. Mennich*  
ATTORNEY

## 1

3,473,900

ALUMINUM-CARBON FIBER COMPOSITES  
Raymond V. Sara, North Olmsted, Ohio, assignor to  
Union Carbide Corporation, a corporation of New  
York

Filed Feb. 21, 1967, Ser. No. 617,662  
Int. Cl. B23p 11/00; B21d 39/00

U.S. Cl. 29—195

8 Claims

### ABSTRACT OF THE DISCLOSURE

Lightweight, strong composite refractory articles comprising a plurality of tantalum coated carbon fibers bonded together by an essentially aluminum matrix are provided. Such composite articles are characterized by a high modulus of elasticity and are especially suited as materials of construction for aerospace and hydrospace vehicles and systems.

### BACKGROUND OF INVENTION

#### Field of the invention

The present invention relates to a composite refractory article which is made up of a plurality of high modulus, high strength carbon fibers which are completely coated with a thin layer of tantalum and bonded together by an aluminum matrix.

#### Description of the prior art

Recently, in the space and missile industries, there has developed a need for materials of construction which exhibit exceptional physical properties, for example, low density coupled with high strength and stiffness. Attempts to produce such materials have centered around the fabrication of composite articles.

One of the most promising materials available today for use in composite form is carbon textiles since they are available commercially in all known textile forms. Today, it is well known to form composites of carbon textiles and resins.

Recently, efforts have been directed to forming composites of carbon textiles and metals. The object of forming such composites is to increase the strength of the metal matrix by the inclusion therein of the high strength carbon fibers.

Aluminum has been suggested as the matrix media for carbon fiber-metal composites which are intended for use in aerospace applications, in the main, due to its low density. However, aluminum does not wet pure graphite for all practical purposes unless aluminum carbide is formed at the interface. Such an aluminum carbide phase cannot be tolerated due to its thermochemical instability.

In order to overcome the inherent lack of wettability of carbon fibers with aluminum, it was decided to try and coat carbon fibers with a thin metallic coating which then would be wetted by aluminum. However, most metals react extensively with aluminum above its melting temperature and form one or more brittle intermetallic phases. The intermetallic constituents or phases either degrade certain mechanical properties of the composite or result in dewetting of the aluminum from around the coated fibers. An extensive study was made of the interfacial zone formed between titanium, chromium, nickel, copper, columbium, silver, molybdenum, tungsten and tantalum respectively, and aluminum to determine which metals are most compatible with aluminum and therefore most useful as intermediate phase-free coupling or wetting agents. Of all the metals tried only tantalum was found to be entirely satisfactory.

## 2

### SUMMARY

Broadly stated, the carbon fiber-aluminum composite article of the invention comprises a plurality of carbon fibers each of which is coated with a thin layer of tantalum and bonded together, preferably in a side-by-side or parallel manner, with an aluminum binder or matrix. Generally, this composite article may be provided by a process which comprises coating carbon fibers with a thin but continuous film of tantalum, compacting the so-called fibers into the desired form, infiltrating the voids between the compacted fibers with molten aluminum and cooling the resultant aluminum infiltrated tantalum coated carbon fibers to produce a composite article. This article can then be formed into any desired shape by known techniques which will readily suggest themselves to those skilled in the art.

### DESCRIPTION OF THE DRAWING

The sole figure shown in the drawing presented herewith is a diagrammatical illustration of a rectangular carbon fiber-metal matrix composite article produced according to the teachings of the instant invention.

Referring now in detail to the drawing, there is shown in cross section a rectangular composite article 1 consisting of aligned graphite fibers 2 having disposed on their surface a continuous one to two micron thick coating of tantalum 3. These so-coated fibers are bonded together by an aluminum matrix 4. The graphite fibers 2 are approximately two inches in length and disposed in the aluminum matrix 4 in a parallel or side-by-side manner. The length dimension of the fibers 2 is perpendicular to surface of the drawing.

### DESCRIPTION OF THE PREFERRED EMBODIMENT OF THE INVENTION

Carbon textiles in any form can be employed in the practice of the instant invention. However, it is preferred to employ carbon fibers in yarn or mono-filament form. Carbon textiles are available commercially and are generally produced by the techniques described in U.S. Patents 3,107,152 and 3,116,975, among others.

Tantalum can be deposited on the carbon fibers by a variety of methods. The techniques available for accomplishing this include electrodeposition from a fused salt bath, thermal decomposition of the appropriate metal halide or sputtering. The exact deposition technique to be employed is dictated by a number of factors. Sputtering can be used on relatively complex shapes and results in a tenacious bond between the thin tantalum coating and the carbon fiber substrate. Such a bond is a highly desirable feature in carbon fiber-metal matrix composites. Thermal decomposition of the appropriate halide requires a heating of the carbon fiber substrate and, accordingly, somewhat limits the type of shapes which can be coated with tantalum in this manner. Electrodeposition of tantalum from a fused salt bath is an ideal way of coating carbon fibers with a thin film of tantalum but this technique is limited to rather simple carbon fiber configurations.

The following example illustrates in detail the preferred practice of the instant invention.

A carbon yarn material which had been heated to graphitizing temperatures was cut into 2 inch lengths. A tantalum coating averaging from 0.2 to 2.0 microns was electrodeposited on these fibers by a technique similar to that described in co-pending U.S. patent application Ser. No. 609,683 which has been assigned to the same assignee as the instant application. These tantalum clad fibers were then placed in an aligned position (all parallel) in a cylindrical capillary tube which was provided with a top and bottom closure. The surface of the cylinder was provided with randomly placed holes or openings to facilitate the

ingress of aluminum into the cylinder and hence into the voids between the aligned carbon fibers. The cylinder containing the carbon fibers in a preselected form was placed into an air tight chamber which also contained a vessel of aluminum. The chamber was then evacuated to a pressure of approximately  $2 \times 10^{-6}$  mm. of mercury to out gas the carbon fibers. The aluminum was heated to a temperature of approximately 700° C. The cylinder containing the aligned fibers was submerged below the surface of the molten aluminum. The chamber was then filled with argon gas to a pressure of about one atmosphere to insure that molten aluminum filled essentially all the voids between the aligned carbon fibers. After about thirty seconds of pressurizing the specimen, the capsule was withdrawn from the molten aluminum, cooled and removed from the chamber.

A metallographic examination of the resultant composite showed that aluminum readily wet the tantalum clad fibers and incorporated them into the matrix without disturbing the tantalum coating and, more importantly, without the formation of a reaction zone at the aluminum-tantalum interface.

Composite so-produced are extremely useful as materials of construction for subsonic and supersonic aircraft, space system components and various propulsion devices.

While the foregoing example concerns a composite where the fibers are positioned in a side-by-side relationship, it is readily apparent to those skilled in the art that the carbon fibers may be randomly orientated in the aluminum matrix if more isotropic physical properties are desired without losing the benefits of the instant invention. In addition, it is obvious that the thickness of the tantalum can be varied as desired. All that is required is that it be thick enough to prevent the aluminum matrix metal from coming into contact with the reinforcing carbon fibers. Likewise, it will be appreciated by those versed in the art that although graphite fibers and fabrics are preferred in the practice of the instant invention, non-graphitic carbon fibers and fabrics may also be employed. Also, other methods of infiltrating the tantalum clad carbon fibers with aluminum will readily suggest themselves to the skilled artisan.

The term carbon as used herein and in the appended claims is meant to include both the non-graphitic and graphitic forms of carbon.

The foregoing example is presented for illustrative purposes only and is not intended to unduly limit the reasonable scope of the instant invention. The limitations of applicant's invention are defined by the following claims.

What is claimed is:

- 5 1. A refractory composite article comprising a plurality of carbon fibers bonded together by an essentially aluminum matrix, said carbon fibers having a continuous coating consisting essentially of tantalum on their outer surface so as to prevent said aluminum matrix from being in direct contact with said carbon fibers.
- 10 2. The composite refractory article of claim 1 wherein said fibers are graphite.
- 15 3. The composite refractory article of claim 1 wherein said carbon fibers are in yarn form.
- 15 4. The refractory composite article of claim 1 wherein said carbon fibers are arranged in a side-by-side, parallel relationship.
- 20 5. The refractory composite of claim 1 wherein said essentially tantalum coating on said carbon fibers is in the range of from about 0.2 to about 2.0 microns thick.
- 25 6. The composite refractory article of claim 2 wherein said graphite fibers are in yarn form.
7. The refractory composite article of claim 2 wherein said graphite fibers are arranged in a side-by-side, parallel relationship.
- 25 8. The refractory composite of claim 2 wherein said essentially tantalum coating on said graphite fibers is in the range of from about 0.2 to about 2.0 microns thick.

References Cited

UNITED STATES PATENTS

|           |        |                       |          |
|-----------|--------|-----------------------|----------|
| 2,683,671 | 7/1954 | Findlay et al. -----  | 29—195 X |
| 2,699,415 | 1/1955 | Nachtman -----        | 29—195 X |
| 2,920,385 | 1/1960 | Fike et al. -----     | 29—195 X |
| 3,098,723 | 7/1963 | Micks -----           | 29—183.5 |
| 3,085,317 | 4/1963 | Stackhouse -----      | 29—194 X |
| 3,384,463 | 5/1968 | Olstowski et al. ---- | 29—191 X |

40 L. DEWAYNE RUTLEDGE, Primary Examiner  
E. L. WEISE, Assistant Examiner

U.S. Cl. X.R.

45 29—197, 198